

April 23, 1935.

E. ROBERTS

1,998,907

INTERIOR PLASTER WALL

Filed Feb. 13, 1932

Fig. 1.



Fig. 2.



INVENTOR  
ELMER ROBERTS  
BY *Walter L. Pipes*,  
ATTORNEY

## UNITED STATES PATENT OFFICE

1,998,907

## INTERIOR PLASTER WALL

Elmer Roberts, Montclair, N. J., assignor, by  
mesne assignments, to United States Rubber  
Company, New York, N. Y., a corporation of  
New Jersey

Application February 13, 1932, Serial No. 592,689

10 Claims. (Cl. 72—123)

This invention relates to interior plaster wall construction and the methods for producing a more flexible interior plastic composition and one which will not have the usual brittleness which invariably results in the formation of a number of small cracks.

Heretofore, it has been common practice to incorporate hair and other fibrous materials in interior plaster wall compositions in an effort to bond the material together and prevent cracking of the plaster wall. The use of such material results in an apparent increased toughness of the plaster composition and generally prevents the plaster from falling after it has cracked. However, no increased flexibility can be obtained by this method and although the plaster is prevented from falling in large pieces after it has cracked, the treatment with hair and other fibrous materials in no way prevents the formation of the cracks themselves in the wall. Sometimes a fabric is applied to the wall surface and the fabric covered wall papered to prevent cracking. Various chemicals have been used in plaster compositions in order to hasten the setting and increase the hardness of the walls, but in none of these methods is an increased flexibility produced nor any appreciable decrease in the tendency of the plaster wall to crack.

Several embodiments of the invention are illustrated in the accompanying drawing, in which:

Figure 1 illustrates a plaster wall over which paper or fabric is applied; and

Fig. 2 illustrates a plaster wall over which a layer of paint is applied.

In carrying out my invention, I apply the plaster wall to a suitable base, with or without the addition of hair, or other fibrous material to the composition, in a manner well known in the art. While the wall is still wet, or, if desired, after it has partly or wholly dried, I apply by spraying, brushing, or spreading an aqueous dispersion of rubber to the wall or ceiling surface. The rubber material may be natural latex or an artificial dispersion of rubber or rubber-like material and may be unvulcanized, or pre-vulcanized, or mixed with compounding ingredients including well known ultra accelerators which will vulcanize the rubber deposit from such dispersion at normal temperatures under atmospheric conditions. It is also desirable to dilute the dispersion to a viscosity permitting ready absorption into the surface of the plaster material, and in order to further aid in the penetration, I may add to the latex composition a wetting or penetrating agent such as sulphonated castor oil, ortho toluidine, Nekal,

or other well known penetrating compositions. Where a wall paper or suitable fabric is to be applied to the plaster surface subsequent to the treatment with the rubber composition, it is desirable to use a thin enough dispersion of rubber so that it will penetrate into the interstices of the wall and not form a continuous film over the surface. In this way, after drying, a reinforcing and flexible web of rubber material acting to bond the particles of plaster together will be formed in the interior of the wall and after the paper or fabric has been applied to the surface by the usual adhesive materials such as flour or starch paste and the like, the wall is still able to breathe through the paper or fabric, as is desirable in this type of construction. Such a structure is illustrated in Figure 1 where a plaster wall 1 that has been treated with an aqueous dispersion of rubber so that the dispersion penetrated into the wall to form a reinforcing web in the interior of the same is covered with a layer 2 of paper or fabric material. However, where the wall is to be subsequently painted with a continuous film of paint, rather than papered, it is perhaps desirable to apply the rubber dispersion so that a continuous film of the same is formed on the surface of the wall. Thus in addition to the rubber penetrating into the plaster wall and forming a reinforcing and flexible web of rubber in the interior of the wall acting to bond the particles together, a continuous film of rubber is also formed on the surface thereof. This continuous film when dried, in addition to increasing the flexibility of the wall, also forms an excellent adhesive base for the paint material applied to the finished wall surface. Such a structure is illustrated in Figure 2 where a plaster wall 3 has been coated with a continuous film 4 of rubber deposited from an aqueous dispersion of rubber and the rubber film 4 covered with a continuous layer of paint 5. In some cases it is desirable to apply a continuous film of rubber dispersion to a wall that is to be covered with paper or fabric and apply such paper or fabric to the wall surface freshly wetted with the continuous film of dispersion prior to drying in order to secure adhesion by a common bond between the paper or fabric and the rubber in the interior of the wall through the continuous rubber film at the surface.

As a specific illustration of one manner of carrying out the invention, without intention to limit the invention except as required by the prior art, the following example is included: To a plaster wall surface either wet, partially dry, or dry, the following composition may be applied

by spraying, brushing, or by some other suitable manner.

|                     | Parts  |
|---------------------|--------|
| Latex (solids)      | 100    |
| 5 Penetrating agent | 2 to 5 |
| Glue                | 3      |
| Ultra accelerator   | 1      |
| Zinc oxide          | 2      |
| Sulphur             | 3      |
| 10 Anti-oxidant     | 1      |

Latex is the rubber dispersion used as an illustration in the above example, and should preferably have a solids content of from 18-25%, although it may, under certain circumstances, vary from 10-60% solids content. The latex may be of normal consistency, or diluted, or concentrated as by evaporation, creaming or centrifuging, and is preferably alkaline with a hydrogen ion concentration of approximately pH 10 to 12, although the hydrogen ion concentration may vary within wider limits as from a pH of 7 to 14. Other aqueous dispersions of rubber, such as artificial dispersions of crude or reclaimed, rubber, or of rubber substitutes or synthetic materials resembling rubber may be used, and it is to be understood that the term "aqueous dispersions of rubber" includes the same. The wetting or penetrating agent if included, may be sulphonated castor oil, ortho toluidine, Nekal, or other well known wetting materials, and the ultra accelerator and anti-oxidant may be any of the well known products now in general use in the art. The rubber dispersion, if desired, need not contain vulcanizing ingredients, in which case the rubber deposit in the plaster wall will not be vulcanized. The treated plaster wall is dried and paper or fabric, or a paint surface applied thereto. With a paint surface, it is desirable to vulcanize the deposit applied to the wall in order to reduce to a minimum any possible residual tackiness of the painted surface. The term "plaster" as used throughout the description and claims is to be interpreted broadly and in addition to ordinary plaster surfaced walls is intended to include stucco surfaces, composition plaster board containing plaster embedded laths faced with card board and plaster compositions containing hair, other fibrous materials, chemicals and the like.

In view of the many changes and modifications that may be made without departing from the principles underlying the invention, reference should be made to the appended claims for an understanding of the scope of the invention.

Having thus described my invention, what I claim and desire to protect by Letters Patent is:

1. In an interior wall construction, a surface comprising plaster having a reinforcing and flex-

ible web of vulcanized rubber acting to bind the plaster particles together.

2. In an interior wall construction, a surface comprising plaster having a reinforcing and flexible web of the solids deposit of an aqueous dispersion of rubber acting to bind the plaster particles together. 5

3. In an interior wall construction, a surface comprising a plaster aggregate, the particles of which are bonded together at least in part by a reinforcing and flexible web of the solids deposit of an aqueous dispersion of rubber, said rubber being vulcanized. 10

4. In an interior wall construction, a surface comprising a plaster aggregate, the particles of which are bonded together at least in part by a reinforcing and flexible web of the solids deposit of an aqueous dispersion of rubber and a layer of paper or fabric over said plaster. 15

5. In an interior wall construction, a surface comprising a plaster aggregate, the particles of which are bonded together at least in part by a reinforcing and flexible web of the solids deposit of an aqueous dispersion of rubber, and a continuous layer of rubber on said surface. 20

6. The method of constructing wall interior which comprises applying plaster to a suitable base and applying an aqueous dispersion of rubber to said plaster to form a reinforcing and flexible web of rubber material acting to bond the particles of plaster together, drying and vulcanizing said rubber. 25

7. The method of constructing wall interior which comprises applying plaster to a suitable base and spraying an aqueous dispersion of rubber on said plaster to form a reinforcing and flexible web of rubber material acting to bond the particles of plaster together. 30

8. The method of improving the flexibility and reducing the cracking tendency of plaster walls which comprises treating said walls with an aqueous dispersion of rubber to form a reinforcing and flexible web of rubber material acting to bond the particles of plaster together. 40

9. The method of constructing wall interior which comprises applying plaster to a suitable base, applying an aqueous dispersion of rubber to said plaster to form a reinforcing and flexible web of rubber material acting to bond the particles of plaster together, and applying paper or fabric to said treated plaster. 45

10. The method of constructing wall interior which comprises applying plaster to a suitable base, and applying an aqueous dispersion of rubber to said plaster to form a reinforcing and flexible web of rubber material acting to bond the particles of plaster together. 55

ELMER ROBERTS.